

Patented June 7, 1927.

## UNITED STATES PATENT OFFICE.

JAMES BROOKES BEVERIDGE, OF RICHMOND, VIRGINIA.

## MANUFACTURE OF PAPER PULP.

No Drawing.

Application filed April 13, 1925. Serial No. 22,884.

This invention has for its object the utilization of the waste liquor from sodium acid sulphite pulp process in the manufacture of pulp by the sulphate of soda process.

5 When wood and other fibrous materials are digested in aqueous solutions of sodium acid sulphite, the waste liquors therefrom contain sodium acid sulphite and sodium sulphonic organic compounds.

10 In the manufacture of pulp by the sulphate of soda process, losses of chemicals occur in the cycle of digesting the fibrous substances and recovery of the chemicals. These losses must be made up by the addition of sodium and sulphur compounds in some form. These fresh chemicals are added in the chemical recovery system.

15 Also in the manufacture of sulphate of soda pulp, it is the general practice to charge the digester with chips, pump in the strong freshly-made alkaline cooking liquor, the volume of which is usually not more than one-half of that required to fill the digester, the necessary volume to cover the chips being made up by the addition of waste "black" liquor from a previous digestion.

20 My process is to make up the necessary volume by the addition of the waste liquor from the sodium acid sulphite process instead of the waste "black" liquor above mentioned. By the addition of this waste acid sulphite liquor, no fresh chemicals will need to be added in the chemical recovery and in the preparation of the cooking solutions for the manufacture of sulphate of soda pulp,

25 which is necessary in the present practice of this process, as the sodium and sulphur present in the waste sulphite liquor is sufficient to make up the chemical and mechanical losses of these two elements occurring in the manufacture. The soda salts in the waste black liquor resulting from the above method of cooking sulphate of soda pulp are then recovered for re-use as is the general practice in the sulphate of soda process.

40 My invention can be carried out in several ways:

- 50 1. After the requisite volume of strong alkaline cooking solution has been pumped into the digester, the volume is made up with waste sodium acid sulphite liquor.
- 55 2. To mix the waste liquor from the so-

dium acid sulphite pulp with the fresh strong alkaline cooking liquor and then pump the mixture into the sulphate of soda pulp digester.

3. To pretreat the chips in the sulphate of soda digester with waste liquor from the sodium acid sulphite pulp and after such pretreatment to drain off a portion, and then add the strong alkaline cooking solution in sufficient quantity to complete the digestion of the fibrous materials into pulp.

What I claim as new is:

1. The method of treating woods and other fibrous substances for the production of pulp which comprises the cooking of the said woods and other fibrous substances in a mixture of sodium hydrate and sodium sulphide in aqueous solution, and of waste liquor obtained from the digestion of woods and other fibrous substances in solution of sodium acid sulphite.

2. The method of treating woods and other fibrous substances for the production of pulp which comprises the pretreatment of the said woods or other fibrous substances with the waste liquors obtained from the treatment of woods and other fibrous substances in aqueous solutions of sodium acid sulphite, and thereafter completing the conversion of the pretreated woods or other fibrous substances into pulp with aqueous solutions containing varying amounts of sodium hydrate and sodium sulphide.

3. The method of utilizing the sodium and sulphur contained in the waste liquor obtained by digesting woods and other fibrous substances in aqueous solutions of sodium acid sulphite comprising the mixing said waste liquor with solutions of sodium hydrate and sodium sulphide, and using this mixture for the manufacture of sulphate of soda pulp.

4. In the process of manufacturing paper pulp by the sulphate of soda process, the step of employing in the digestor in combination with the liquor used in the sulphate soda process, waste liquor resulting from the digesting of wood or other fibrous material with sodium acid sulphite.

In testimony whereof I hereunto affix my signature.

JAMES BROOKES BEVERIDGE.